

J. B. WALKER.

PROCESS FOR PRODUCING SOLID CASTINGS AND THEIR PRODUCT.

APPLICATION FILED JAN. 22, 1918.

1,294,209.

Patented Feb. 11, 1919.



Fig. 3.



Fig. 4.



Fig. 2.



Fig. 1.

Inventor

JOHN B. WALKER

Witness

J. Gordon Parker

By

Thomas Johnston

Attorney

# UNITED STATES PATENT OFFICE.

JOHN B. WALKER, OF BIRMINGHAM, ALABAMA.

## PROCESS FOR PRODUCING SOLID CASTINGS AND THEIR PRODUCTS.

1,294,209.

Specification of Letters Patent.

Patented Feb. 11, 1919.

Application filed January 22, 1918. Serial No. 213,136.

*To all whom it may concern:*

Be it known that I, JOHN B. WALKER, a citizen of the United States of America, residing at Birmingham, in the county of 5 Jefferson and State of Alabama, have invented certain new and useful Improvements in Processes for Producing Solid Castings and Their Products, of which the following is a specification.

10 My invention relates to a new and improved method of casting ingots and castings so as to reduce to a minimum the defects in the body of the casting due to gas pockets, piping and the like which may generally be said to result from the chilling and hardening of the outer walls of the casting while its core and center is still molten so 15 that the gases generated in the casting become trapped to form therein gas pockets 20 and the molten core as it chills and contracts shrinks away from the casting walls and leaves a large pipe or cavity.

My process, in its broadest sense, contemplates the removal of the gases from within 25 the casting during the period it is solidifying by means of an artificial vent or flue which penetrates the casting's frozen outer wall so as to permit the gases trapped therein to escape freely from the hot center of 30 the casting as it gradually cools. I cause this vent, when formed by an inserted flue, to extend sufficiently below the frozen top or outer wall of the ingot or casting to exhaust the gases, the depth of penetration of 35 the flue being empirically determined with due regard to the size of the casting and the character of the metal. Such a vent flue is the simplest means to the ends I have in view and may be of any character which 40 can be cheaply and readily introduced into the top of the ingot or into the head or gate of a casting before it chills and which will resist any tendency of heat of the casting to destroy its venting functions. I have also 45 discovered that if certain materials such as limestone, fluorspar, thermit and like reagents which have the effect of intensifying the heat and fluidity of the molten metal with which they are brought into contact, 50 are introduced into the casting, they will cause an internal reaction which will vent the casting and raise its internal temperature to a point where the tendency to pipe is brought under control and if this reac-

tion is used with the artificial vent flue the 55 piping may be practically eliminated.

In experiments which I have conducted with high carbon steel ingots I have caused the top of the ingot about the vent flue to collapse so that the pipe or shrinkage cavity was practically eliminated. A wide variety of reagents, the properties of which are well known to those skilled in this art, may be employed to the ends above described and may be introduced in a very simple and 60 practical manner by placing them in the lower closed end of a pipe or flue, the main portion of which may be left open or filled with material suitable for preserving the 65 venting functions of the flue.

70 My invention further contemplates the reduction to a minimum of the metal in the heads of castings so that the maximum percentage of cast metal will be available for the production of finished products and to 75 this end the venting flue is so introduced into the head that should the pipe occur in the casting it will be drawn up into the head and will leave the main body of the casting solid. To illustrate this feature of 80 my invention I have cast steel rolls weighing from eight to twelve tons with heads reduced from three feet to less than two feet and have found the piping greatly reduced and wholly confined to the short head, 85 the roll proper being entirely free from cavities or gas pockets.

85 The simplest and least expensive method of carrying out my invention is illustrated in the accompanying drawings, in which:— 90

Figure 1 is a sectional view illustrating a high carbon steel ingot as produced by the present casting methods.

Fig. 2 shows an ingot mold in vertical section with an ingot poured therein and my 95 improved vent at the moment it is moved into operating position.

Fig. 3 illustrates the finished ingot in section after it has hardened and shows how a vent flue formed of metal pipe is melted 100 away to release the reagent and open the vent flue.

Fig. 4 illustrates another form of vented casting after treatment with my fluxing and venting process.

Similar reference numerals refer to similar parts throughout the drawings.

As illustrated, 1 is an ingot mold of any

standard type and the molten metal to form the ingot 2 has been poured into the mold in any manner as customarily practised in this art. At the completion of the pouring 5 operation and preferably before the top of the ingot has chilled or frozen, I introduce an artificial vent or flue formed preferably by a short length of thin metal pipe 3, but any other material which will not injuriously 10 affect the ingot or casting may be used. This pipe at its upper end has a handle 4 clamped thereto and at its lower end is pinched together at 5 so that it forms a container for a filling, if such is desired, 15 of material which will resist the heat of the casting so that it will not solidify and prevent the escape of gases through the pipe flue. This material should be such as not to injuriously affect the ingot or casting 20 when coming in contact with its molten metal. In practice, I have charged the pipe with lumps of slag or limestone and alumina, or dolomite, but any refractory materials, preferably such as will not take up 25 carbon, may be substituted. The handle 4 is so placed as to come to rest on the mold 1 when the lower end of the pipe penetrates the desired distance into the casting.

It will at once be apparent that the cool 30 wall of the pipe 3 will chill the casting metal about it and freeze the pipe or vent flue in position with its lower end entering the molten interior of the casting. This end 5 will melt away leaving fixed in the 35 upper end of the ingot a vent stack or open flue of material which will not conglomerate and through which the contained gases in the casting can escape and thus prevent gas pockets forming and reduce to a controlled 40 minimum the piping loss in ingots. I have found that excellent results are obtained where a vent stack of four inch iron pipe is caused to penetrate a six ton steel ingot about twelve inches as this will carry it well 45 below the depth of the frozen top zone of the ingot and it thus leaves the lower open end of the stack in communication with the slowly cooling molten center of the ingot where the generation of the gases is continu- 50 ously proceeding as the ingot cools.

To obtain the best results from my process the vent pipe should be utilized as a preferred means to introduce into the casting a reagent or flux of such character as to 55 intensify the internal heat of the casting about the base of the flue and increase the fluidity of the molten metal to facilitate the liberation of its gases. As shown in Fig. 2, I place at the lower end of the pipe 3 sufficient fluxing material 6 such as thermit, fluorspar, limestone and the like which 60 serves to so increase the internal temperature at the top of the ingot or casting as to practically eliminate the pipe, it being 65 possible to cause the top of the ingot to

sink down, as shown in Fig. 3, and contract, and in many cases fill, the pipe space with solid metal. As illustrative of this phase of my invention, I inserted five pounds of thermit into a four inch iron pipe and 70 thrust it twelve inches into a large ingot. The upper end of the ingot turned to a white heat and gases were driven off through the vent pipe for fifteen minutes.

In Fig. 4 I show my invention applied 75 to foundry practice wherein a roll casting 7 is shown with the pipe 3 inserted about ten inches into its head 8. A three and one-half inch pipe was used here with about four pounds of thermit and the pipe 9 was 80 found to be drawn entirely into the head, leaving the casting solid. I have also thrust my artificial vent flue into the gates of many large castings and freed them entirely from 85 blow holes or gas pockets.

It is within the scope of my invention 90 that the vent pipe may be used without the reagent, and the reagent may be introduced into the casting in any suitable manner with beneficial results, but I have obtained the best results from the joint use of both vent pipe and reagent. Moreover, the artificial 95 vent flue may be of any shape or material so long as it is capable of becoming frozen in place in the casting and is adapted to preserve its venting functions during the cooling of the casting.

As my invention thus produces a different and distinct type of casting, I desire 100 to claim also, as a part of this invention, the product of my process. Fig. 1 shows a typical high carbon steel ingot cast by the present processes with its blow holes or gas pockets and its large pipe 9.

Where the thermit or like reagent is used 105 in the pipe it is not necessary to fill the latter with the refractory bodies, but it is essential, otherwise, to employ some medium to maintain the venting functions of the pipe or vent flue.

Having thus described my invention, what 110 I claim as new and desire to secure by Letters Patent is:—

1. The herein-described process for the production of solid castings, which consists in 115 providing a vent pipe of material fusible in the internal heat of the casting to be vented and having one end of the pipe closed and causing said closed end of the pipe to penetrate substantially into the molten interior of the casting and to be melted away after the pipe is frozen in place in the casting.

2. An ingot or casting having incorporated therein a pipe forming an artificial 120 venting flue composed of material which will fuse in the internal heat of the casting and which penetrates into the portion of the casting's interior that last solidifies and filling the outer portion of said pipe with 125

bodies of material that will not agglomerate in the heat.

3. An ingot or like casting having incorporated in the upper portion thereof an artificial vent formed of a flue and containing refractory bodies and having its inner end melted away.

4. A casting having a venting flue of a metal pipe filled with a reagent and penetrating below the initial chilled zone at the top of the casting.

5. The herein-described process for the production of solid ingots and castings, which consists in providing a vent flue of material fusible in the internal heat of the casting, closing one end of said flue, introducing an active reagent in the closed end of the flue, charging bodies of material in the flue above the reagent of such character that they will not agglomerate in the heat of the casting, and causing the closed end of the flue to penetrate through the upper crust of the casting into its molten interior so that the closed inner end containing the active reagent will melt away and release the reagent while its outer end containing the other material is frozen in place.

6. The herein-described process for the production of solid castings, which consists in providing a metal pipe with one end closed, introducing thermit into said closed end of the pipe, filling the rest of the pipe with calcareous bodies, causing said closed end of the pipe to enter into and be melted away by the molten interior of the casting while the outer end of the pipe is exposed for venting by the occluded gases, substantially as described.

7. The herein-described process for casting solid homogenous ingots and castings, which consists in penetrating the frozen crust of the solidifying ingot with a vent pipe of material fusible in the casting and containing at its inner end a reagent such as ther-

mit which is liberated into the molten interior of the casting when the inner end of said pipe fuses.

8. The herein-described process for the production of ingots and castings, which consists in introducing into the top of the ingot or casting before it hardens a fusible pipe open at its outer end and closed at its inner end and containing a reagent adapted to be brought into contact with the molten interior of the casting by the melting of the inner end of the pipe.

9. The herein-described process for the production of ingots and castings, which consists in introducing into the molten casting a fusible metal pipe closed at its inserted end and filled with a reagent, the pipe being adapted to form a venting flue which remains frozen in place in the ingot after the melting away of its inner end to charge the reagent into the body of the ingot, and which serves to vent the gases from the molten interior of the ingot until the latter chills, substantially as described.

10. The herein-described casting process, which consists in introducing fluxing materials into the molten interior of the casting and maintaining by means of a pipe frozen in place in the casting a vent through the frozen outer wall of the casting to carry off the contained gases.

11. The herein-described process for the production of solid castings, which consists in maintaining a venting flue penetrating the top chilled zone of the casting and bringing into contact with the molten interior of the casting a fluxing material to intensify the heat and increase the fluidity of the molten interior of the casting adjacent to the inner end of the vent.

In testimony whereof I affix my signature. 85  
JOHN B. WALKER.

Witness:

NOMIE WELSH.